

Nov. 3, 1959

L. K. SCHUSTER ET AL

2,911,332

PROCESS OF COATING METAL AND RESULTING ARTICLES

Filed May 25, 1956



Fig. 2



LUDWIG K. SCHUSTER &  
ALFONSO L. BALDI JR.  
INVENTORS.

BY *Connally and Tracy*

THEIR ATTORNEYS

# United States Patent Office

2,911,332

Patented Nov. 3, 1959

1

2,911,332

## PROCESS OF COATING METAL AND RESULTING ARTICLES

Ludwig K. Schuster, Philadelphia, and Alfonso L. Baldi, Jr., Drexel Hill, Pa., assignors, by mesne assignments, to Kelsey-Hayes Company

Application May 25, 1956, Serial No. 587,388

13 Claims. (Cl. 148—6.2)

This invention relates to the coating of metals, for the purpose of improving their corrosion resistance as well as the adhesion of organic top coatings such as paints, lacquers, or resins in general.

Among the objects of the present invention is the provision of novel coated metal products that are simple to manufacture and of outstanding characteristics, as well as the provision of methods for applying the coatings.

The above as well as additional objects of the present invention will be more completely understood from the following description of several of its exemplifications, reference being made to the accompanying drawing in which Fig. 1 shows an aluminum wire coated in accordance with the present invention, and Fig. 2 is a partially broken away view of a container made from coated metal and illustrative of the present invention.

According to the present invention, a metal face is coated with an aqueous solution essentially of chromic acid and a compatible reducing agent for the chromic acid, and the coated surface is heated to a temperature of from 250 to 500 degrees F. to cause the reducing agent to react with the chromic acid and leave a water-insoluble layer, the proportions of reducing agent and chromic acid being such that from about 40 to about 95% of the chromium in the chromic acid is reduced to trivalent form, and the final layer weighs at least about 3 milligrams per square foot of surface. With metals such as zinc, cadmium, magnesium and aluminum, considerably better results are obtained when the coating weight is above 10 milligrams per square foot.

The reducing agent is preferably one that does not leave water-soluble salts in the final coating layer. Compatible reducing agents are those that when present in the above proportions do not cause any precipitation during the period in which the solution is kept as a solution, and are not driven off by the heat treatment before they are oxidized. Organic polyalcohols are very effective reducing agents, and examples of specifically desirable polyalcohols include sucrose, invert sugar, dextrose, glycols, polyglycols such as diethylene glycol, glycerine, mannitol, sorbitol, triethanolamine and tartaric acid. Other reducing agents such as citric acid and hydroxylamine salts, such as hydroxylamine sulfate and even phosphorous acid are also suitable. Although reducing agents such as potassium iodide and phenol can be used, they produce coatings that are not too satisfactory. The reducing agent should not be so stable that it cannot be oxidized by the chromic acid, at least when it reaches the final baking temperature. A coating bath containing both the chromic acid and the reducing agent should not be permitted to stand long enough to form deposits of insoluble chromium compounds before the bath is applied to the surface and cured, that is, subjected to the final heat treatment. To avoid this, the dwell of the reducing agent in contact with the chromic acid solution should be of limited duration. The chromic acid and the reducing agent can even be applied as by spraying from a com-

2

mon spraying jet, solutions of the separate ingredients being mixed together only just before spraying.

The reducing agents listed above do not react very rapidly and can be stored in a chromic acid solution for at least one day at room temperature (80° F.) without deterioration.

In general, polyalcohols and their oxidation products are suitable reducing agents. These contain a carbon atom to which is linked an alcohol group that is not protected against oxidation, and such structure appears to be effective regardless of the remainder of the molecule, so long as the materials are not too volatile.

The presence of volatilizable material in the coating bath in general does not detract from its efficacy, if it does not interfere with the reducing operation. In fact, some additives such as ammonia appear to improve the corrosion resistance and lacquer-adhesion of the coating on tin-plated steel for instance. The addition of ammonia can for example be made to the point where the CrO<sub>3</sub>-reducing agent bath is rendered slightly alkaline (pH 7.4 for example), although greater or lesser additions of ammonia are also helpful. A suitable pH range is from 3 to 10. The addition of ammonia is most significant when coatings weighing less than 10 milligrams per square foot are applied.

The concentration of the components in the coating solution will depend upon the weight or thickness of the coating desired—the heavier coating requiring the use of the more concentrated solutions. The ratio of the chromic acid to the reducing agent will vary, depending upon the reducing agent selected, but such a ratio should be used that 40 to 95% of the total chromium is reduced to the trivalent condition in the final coating. For sucrose an effective range is 1/1 to 8/1 and preferably 2/1 to 5/1 by weight. The percentage of trivalent chromium in the coating can be determined by dissolving it in a 2-40% aqueous solution of NaOH by weight heated to 160° F. or higher, titrating the hexavalent content of the resulting solution with sodium thiosulfate, and subtracting this from the total chromium content which is determined by oxidizing another dissolved coating sample with H<sub>2</sub>O<sub>2</sub> and again titrating with sodium thiosulfate.

The greater the trivalent chromium content, the more insoluble the coating and the more resistant it becomes to chemical attack. However, the greater resistance to attack requires longer treatment for dissolution of the coating in the above analytical procedure. When the coating is applied over zinc, aluminum or other metal soluble in caustic alkali, the hexavalent chromium content is reduced during the dissolving step by the chemical action on the metal. Apparently the nascent hydrogen generated by the action effects the reduction. The hexavalent chromium content that any coating bath provides on such reactive metals, can be determined by applying the coating bath in exactly the same way to an alkali-resistant metal, or to surfaces like glass which do not interfere with the analysis, since glass even if attacked by alkali does not appear to cause any change in the hexavalent chromium content. Coatings on glass can be dissolved in more concentrated alkali, such as those containing 40% NaOH by weight. The coating formed on glass appears to be identical to that formed on metal.

The aqueous chromium-oxide-depositing film applied to the metal surface in accordance with this invention is converted to a water-insoluble solid when it is subjected to a temperature at least as high as 250° F. Only a fraction of a second is required for the conversion after the converting temperature is reached. However, some time may be required to reach that temperature, depending upon the rate at which heat is supplied, the thickness and mass of metal, and the heating technique. Any source of heat is applicable. The selection depends upon the

desired conversion speeds, the shape and thickness of the article being heated, etc. Suitable heating sources are, for instance, infra red lamps, cup-type ceramic or tubular metal gas burners heated to incandescence, flames as with ordinary gas burners, induction heating, hot air and the like.

Somewhat better coatings are also obtained if the coating is cured at the higher temperatures and with some metals like zinc, if the curing treatment is prolonged as for example to 5 or 10 seconds or even longer. However, since commercial requirements are for high speed treatments (for instance 600 to 1000 feet per minute), it is most practical to apply the mixed chromium oxide while the metal is moving at that speed. For this purpose the conversion can be arranged to take place almost instantaneously by using heat sources at higher temperatures which brings the aqueous film rapidly to 400° F., for example. Longer cures are effected at these high speeds by using longer curing ovens or burners.

The coating solution can be applied by immersion, flooding, spraying, roller coating, etc. Roller coating or spraying is particularly suitable for continuous coating of tin plated strip. The thickness of the coating depends upon the concentration of the solution. If applied by roller coating, the roll pressure and roll surface characteristics also affect the thickness of the final coating.

For commercial applications it is desirable to continually monitor the chromium oxide coating, as for example to make sure it has the desired thickness or weight. Over a magnetic base, such as on tin-plated plain carbon steel, the thickness of the coating, which is non-magnetic, inserts a correspondingly varying reluctance in a magnetic circuit that extends through the coating. Any convenient kind of magnetic reluctance measuring apparatus, such as that shown in U.S. Patent No. 2,703,384, granted March 1, 1955, can be used.

It has been found advantageous to incorporate in the coating solution a small amount of wetting agent on the order of .005 to 0.3% by weight to improve the wettability of the metal surface by the coating solution. With such a wetting agent in the treating solution, the surface of the metal is more uniformly and more rapidly wetted so that the entire treatment time is held to a minimum. The final coating is also more uniform and precleaning problems are minimized. Furthermore, oxidizable wetting agents such as are formed by condensing 3 mols of ethylene oxide with p-(n-octyl) phenol, as described in U.S. Patent No. 2,115,192, may be used to take the place of some of the reducing agent. Long-chained alkyl sulfates are suitable and tertiary butyl alcohol will be effective although it does not cause any appreciable reduction and is generally required to be in higher concentration, e.g. 0.5%, to be really effective. In general, however, anionic, cationic or non-ionic wetting agents including quaternary ammonium compounds of long-chain alkyl or aralkylamines, can be used.

Another feature of the present invention is that the coating does not interfere with welding. No localized removal of the coating is necessary and resistance welding can, for example, be conducted in the normal way used for uncoated metal.

The coating of the present invention can be applied to the surface of any metal to improve the corrosion resistance and paint or lacquer adhesion. The improvements are particularly striking, however, with non-ferrous surfaces such as aluminum and zinc. Other metals that are highly suited for coating include cadmium, copper, silver, magnesium, beryllium, titanium, tin, lead, bismuth, tungsten, cobalt, nickel and alloys of these metals with each other. With tin surfaces the coating of the present invention is preferably used with coating weights less than about 10 milligrams per square foot to provide the best adhesion of organic finishes, such as paints, enamels or lacquers. Tin platings on other metals, such as plain

carbon steel, are greatly improved by the coating of the present invention.

A feature of the present invention is that the coating is particularly highly resistant to alkaline attack. Metals like aluminum are in some uses quite vulnerable to such attack, as for example, when used in the form of conductor wire of telephone and power supply circuits.

Fig. 1 shows such a wire 6 made of 99.99% aluminum with the coating 8 of the present invention covering it. Such a wire can be laid in underground cables and exposed to the air or the weather without any detectable attack on the aluminum for extremely long periods of time.

Fig. 2 shows a can 10 representing another embodiment of the present invention. The can has a tubular body 12 made in the conventional manner from a single strip of SAE 1010 steel 31, 10 mils thick plated with a layer of tin 32, that is covered with a coating 34 according to the present invention. The ends of the strip are joined together as indicated at 13. These ends are folded back on each other to provide interlocking flanges 16 and 18 between which a yielding gasketing layer 17 such as rubber is applied. The flange and gasket combination is then crimped together to make a suitably sturdy and leak-proof joint.

The openings at the top and bottom of the tubular body are sealed with covers 20, 22 that have beaded peripheries 24 with interlocking flanges 26, 28. The interlocking beaded periphery can merely be crimped in place, preferably with a layer 30 of gasketing to assure hermetical sealing.

The following specific examples show some of the ways in which the present invention can be practiced.

#### Example I

Clean a sheet of 24ST aluminum by dipping in an aqueous solution of 5 ounces per gallon of sodium metasilicate and  $\frac{1}{2}$  ounce per gallon of disodium hydrogen phosphate held at 160 to 170° F.

Rinse the cleaned metal in tap water at 70° F.

Dip coat the rinsed metal in an aqueous solution containing  $2\frac{1}{2}$  CrO<sub>3</sub>, 0.83% triethanolamine and 0.005% of the wetting agent formed by condensing 3 mols of ethylene oxide with p-(n-octyl) phenol as described in U.S. Patent No. 2,115,192, the solution being held at 70° F.

Roll the coated metal through rubber rollers wetted with the coating solution.

Cure in an air furnace held at 1700° F. by passing the rolled sheet through with a dwell of 15 seconds in the furnace so that the peak temperature of the aluminum surface reaches 400 to 450° F.

The adhesion of organic coatings such as paint to the resulting surface is extremely good and the unpainted coated aluminum sheets show almost no corrosion after standing out in the weather for six months. The paint or lacquer adhesion is even further increased by mechanically or chemically roughening the aluminum surface before the mixed chromium oxide layer is applied. Wire brushing, sand blasting, slurry blasting, or chemically etching will provide an excellent paint bonding surface even though the mixed chromium oxide layer intervenes. An effective chemical etching operation is one carried out in an aqueous solution of 5 ounces per gallon of sodium hydroxide and 0.1% of a wetting agent such as isopropyl naphthalene sodium sulfonate or the wetting agent described in Example I. Removal of about 300 to 4000 milligrams per square foot of aluminum gives very satisfactory results.

#### Example II

A 24 mil thick round wire of 3S aluminum was passed in a continuous manner through the following treatment condition:

(1) Three seconds in an etching bath of 10% NaOH and 3% sodium gluconate in water held at 160° F.

- (2) One second rinse in tap water at 70° F.  
 (3) Two seconds in 5% HNO<sub>3</sub> by weight in water at 70° F.

(4) One second rinse in tap water at 70° F.

(5) One second in an aqueous solution of 8% CrO<sub>3</sub> by weight and 2.7% sucrose by weight.

(6) Three seconds cure in an air oven having an internal temperature of 1200° F., the wire surface reaching 400° F.

The resulting coated wire has a coating of 85 milligrams per square foot and an unusually high resistance to attack by alkali, showing a ten-fold increase in resistance to 0.1 N NaOH as compared to untreated wire. The alkali resistance of the mixed chromium oxide coatings is best when the coatings are cured at temperatures of 400° F. or higher and when the coating weights are above about 20 milligrams per square foot.

As shown in prior application Serial No. 458,668, filed September 27, 1954, and now abandoned, the coatings of the present invention are also helpful in covering zinc surfaces such as those made by electroplating or hot dipping plain carbon steels with zinc. Without this protection the zinc rapidly develops "white rust," particularly on standing in a humid atmosphere. The disclosures of the prior application is hereby incorporated herein as though fully set forth.

The adhesion of some paints, enamels and lacquers to the mixed chromium oxide coating on zinc is markedly increased when the curing temperature is raised to between 400 to 500° F. The popular melamine-modified alkyd paints or unmodified alkyd paints described in Paint and Varnish Technology by Von Fischer, published 1948, chapter 9, pages 127-144, for example, adhere unusually well to a mixed chromium oxide coating which has been heated above 400° F., even though the paint itself is cured at 350° F. or below. However, the adhesion of this paint is not as good as phenolic, oil-modified alkyd, or oleoresinous paints when the mixed chromium oxide coating, either before or after the application of the paint, is not heated as high as 400° F. Paint-covered coatings do not have the corrosion problems of zinc filmed with uncovered mixed chromium oxides, and when a paint is to be applied there is no significant advantage in having the mixed chromium oxide layer cured for more than one or two seconds.

The adhesion of the mixed chromium oxides to the zinc is so great that it can be used to improve the adhesion of the oxide coating on iron or steel. Thus, a flash plating of zinc weighing only about 0.1 to 0.5 pound per base box, can be deposited as from a potassium zinc cyanide bath on plain carbon steel such as SAE 1010, and provides a surface to which mixed chromium oxide coatings of 5 to 200 milligrams per square foot adhere very tenaciously. The resulting metal is highly suited to fabricating operations as in the manufacture of hermetically sealed cans, with or without an additional paint, enamel or lacquer coating. The paint, enamel or lacquer adheres very well to the oxide coating, so that the well-known paint-bonding difficulties of zinc surfaces are also avoided. Cans made in this way are highly suited for holding detergents, paints, etc.

Inasmuch as zinc surfaces are not too easily wetted, as for example when the liquid film that deposits the mixed chromium oxides is applied, it is preferable to always use wetting agents as indicated above, and even to bring the wetting agent concentration to 0.02% or even higher. Furthermore, the use of reducing agents like triethanolamine helps improve the wetting action and is preferred with or without the addition of conventional wetting agents.

By way of example, one highly effective coating bath for zinc electroplated from either potassium zinc cyanide

or acid zinc sulfate baths, or even dip-galvanized surfaces, is a water solution of the following by weight:

*Example III*

5 2% CrO<sub>3</sub>  
 0.6% triethanolamine  
 0.005% of the condensation product of 3 mols of ethylene oxide with p-(n-octyl) phenol as described in U.S. Patent No. 2,115,192

10 No appreciable contact time is needed and the conversion can be effected at 400-500° F. for one second when a paint, enamel, lacquer, etc., is to be applied over it. This treatment used with 0.014 inch thick cold rolled SAE 1010 steel having a 0.9 to 1 pound per base box (approximately 0.000055 inch thick) electroplated zinc surface, makes a product particularly suitable for Venetian blind slats, housings and other accessories. The zinc coating can be applied before the metal is cut to size and shaped, inasmuch as the zinc seems to smear over cut edges and the thin zinc layer is not loosened by fabricating operations. The mixed chromium oxide coating can also be applied before cutting and shaping, and if desired, even the paint can be coated on the oxide layer before these operations.

15 20 An additional feature of the present invention is the cooperation of the mixed chromium oxide coating with a tin underplating, particularly where the tin plating is less than  $\frac{3}{4}$  pound per base box. Such a plating covered by a coating of the present invention weighing between about 5 and 10 milligrams per square foot is exceptionally effective in preventing attack of plain carbon steels, such as those used in cans, as illustrated in Fig. 2.

25 25 The coating is ideally suited for continuous application in high speed tinning operations. Over the coating there can also be applied a layer of enamel, paint, resin or the like, such as those conventionally used to line container walls. An organic layer of this type is very adhesively held in place. It will, for example, remain firmly anchored even when subjected to severe forces such as by having the organic-layer-carrying metal subjected to impact or to a drawing operation.

30 30 As the weight of the mixed chromium oxide layer is reduced below 10 milligrams per square foot, the proportion of reducing agent can usually be diminished, and at a coating weight of about 5 milligrams per square foot, the reducing agent may be eliminated altogether. However, even with minimum coating weights, the use of some reducing agent is advisable to insure the complete 35 insolubility of the heated coating.

35 40 The mixed chromium oxide of the present invention will keep the surface of heavy tin layers, those weighing more than  $\frac{3}{4}$  pound per base box, brighter longer and is desirable for this purpose. The most effective use of 45 50 the chromium-containing coating is with tin platings no heavier than about  $\frac{3}{8}$  pound per base box. Although any corrodible steel can be so covered, plain carbon types (less than about 2% alloying metals) are least expensive and accordingly most desired. They can have a carbon content varying from extremely low values, 0.05% or even less, to as much as 1.4% or higher. The phosphorus and sulphur contents can range from substantially zero up to several tenths of a percent. Generally phosphorous maxima are about 0.15% and sulphur maxima about 0.3%. These materials include the steels ordinarily considered as carbon steels (SAE 1010 to 1095), free cutting steels, plain carbon tool steels, including those that have up to several percent of silicon, and casting 55 60 65 metals.

70 75 The tin plating of the present invention can be applied either electrolytically or by the hot dip process. The lighter platings, however, are much more readily applied electrolytically and electrolytic platings appear to respond better to the presence of the mixed chromium oxides in the coating directly above them. Any type of electrolytic

plating technique can be used with either acid or alkaline plating baths.

The advantages of the present invention are obtained when the mixed chromium oxide coating is applied over the tin plating, whether or not the tin plating is fused. In other words, the final fusing operation normally carried out to flow electrolytically deposited tin plate and thereby change it from a matte to a shiny surface, can be omitted, or can be carried out during the final heating operation in which the mixed chromium oxide coating is cured.

It is also desirable, before applying the chromic acid solution on tin-plated plain carbon steels, to etch the surface of the plated steel with aqueous nitric acid or ferric nitrate. One to twenty percent solution of either or both of these materials will provide a beneficial etch in from 2 to 20 seconds at a temperature of from 60 to 150° F.

In the following examples the final coated products show a great improvement over untreated or otherwise treated tin surfaces in resisting pin-point rusting. This can be illustrated by a hot water immersion test, as for example after immersion in water at 200-212° F. for five hours and seventeen hours at 70° F., untreated tin-plated steel surfaces show severe pin-point rusting while the same tin-plated steel treated as disclosed in any of the examples, showed only slight and localized pin-point rusting.

#### Example IV

A roll of strip SAE 1010 steel 10 mils thick with a  $\frac{1}{4}$  pound per base box electrolytic tin plating from acid stannous sulphate bath, was heated at 470 degrees F. by passing the sheet through a heating chamber composed of incandescent ceramic cups. The tin plating was fused by this treatment. The fused tinned surface was then flooded with an aqueous solution containing 5 grams per liter of chromic acid and  $\frac{1}{2}$  gram per liter of triethanolamine, the solution being held at 80° F. The flooded metal is rolled through resilient rubber rolls wetted with the same solution and then carried between sets of incandescent ceramic gas burners, where it is kept 1½ seconds, the metal temperature reaching 300° F. for about  $\frac{1}{2}$  second. The metal is immediately rolled up into coils. The resulting coating weight is 5 milligrams per square foot.

#### Example V

The procedure is the same as Example IV except 0.6 gram per liter of  $\text{NH}_3$  is added to the chromic acid bath to bring the pH to about 7 to 7.5. The bath now contains  $(\text{NH}_4)_2\text{CrO}_4$  plus a slight excess of  $\text{NH}_4\text{OH}$ . The resulting coated product is particularly adherent and resistant to loosening under deformation or impact.

#### Example VI

The procedure is the same as Example V except 0.75 gram per liter of sucrose is used instead of the .5 gram per liter triethanolamine and a peak curing temperature of 350° F. is used.

#### Example VII

The procedure is the same as Example IV except 1.5 grams per liter of triethanolamine are used.

#### Example VIII

Same as Example V except that the tin is electro deposited in an alkaline sodium stannate bath and only sufficient ammonia is added to bring the pH to about 2.5.

#### Example IX

Same as Example VII except that the pH is adjusted with  $\text{NH}_3$  to 5. This coating showed practically the same unusual adhesion as the coating of Example IV.

#### Example X

Same as Example VIII except that the pH is adjusted with  $\text{NH}_3$  to 8.5.

#### Example XI

Same as Example IV except that the tin is not flow melted after electro-plating and the chromate treatment is applied to the matte tin surface.

Hot dipped tin coatings are also improved by the treatment of the present invention, and retain their shininess or luster much better under humid conditions.

The coatings of the present invention exhibit their outstanding corrosion resistance even without the help of a superficial film of oil. However, such an oil film improves the lubricating of the metal and is advantageously used where the metal is to be handled. Cotton-seed oil, palm oil, or any glyceride oil is particularly desirable since it contributes an unusually large increase in corrosion resistance, and only about 1 milligram per square foot is sufficient. Such a small amount of oil does not interfere with the adhesion of a paint film applied directly over it.

The pre-etching with nitric acid, as described above, is suitable for use with hot dip tin coatings, or electroplated coatings that are fused or unfused. Such etching will give some improvement when carried out on the tin-plated surface but it will also whiten the tin surface and sharply reduce its luster. It is accordingly preferred to do such etching before the tin plating or before the fusion.

The nitric acid etch path is preferably kept at 70-80° F. or below. Above 80° F. it generates so much heat, apparently by oxidizing some bath ingredients, that its temperature can rise to the point of liberating large quantities of  $\text{NO}$  and  $\text{NO}_2$  fumes. Acid temperatures lower than 60° F. generally produce etching very slowly and are accordingly not preferred.

Where preliminary etching is to be carried out on unplated steel used in making food cans or the like, it is even more desirable to monitor the etching operation as by continually inspecting the etched surface. Steel used for other purposes seems to behave about the same even when several thousand milligrams are etched away per square foot. The etching is preferably just sufficient to clearly expose the grain boundaries at the metal surface. This usually takes not more than about 400 milligrams per square foot of metal removal. Ordinarily the removal of at least about 100 milligrams per square foot is needed for best corrosion resistance, but 200 or more milligrams of metal removal per square foot gives better results with mixed oxide coatings of from 5 to 20 milligrams per square foot, with or without the intervening tin layer.

The continuous inspection of such surfaces can be carried out even while the surfaces are moving at the high speeds of commercial operations, by electronically scanning an optical image of the surface on a television pick-up mosaic with a cathode ray beam, and using the resulting electrical impulses to reconstitute an optical duplicate of the image, suitably magnified as desired. In other words, a television camera can be focussed on the surface and used with a television receiver.

The metal surface, even though moving at high speed, can have its image readily scanned by a transversely moving cathode beam that travels fast enough to place successive scanning lines fairly close together and thereby provide the desired degree of definition, 30 to 200 lines per inch, for example. The forward motion of the image can, in fact, be used to supply the entire spacing between the scanning lines so that the transverse scanning need not have any forward component whatsoever. Electrical pick-up signals can then be provided with scanning pulses directed longitudinally with respect to the image motion so that the successive transverse scanning lines will appear as a side-by-side sequence having a predetermined number of lines and then will return for another cycle of such lines. For comfortable observation, the reconstituted image can be formed of only one

longitudinal scanning cycle every few seconds, with nothing appearing in the intervening picture cycles. An occasional raster of this type projecting on a fluorescent screen having a relatively long persistence, will appear stationary and can be conveniently examined for the appearance of the etched surface.

Suitable organic layers for use in the present invention are those usually loosely referred to in the art as enamels, sanitary enamels or lacquers such as the oleo-resinous phenolic or vinyl resin varnishes. Particularly effective forms of such organic type coatings are described in U.S. Patents Nos. 2,231,407, 2,299,433, 2,479,409 and 2,675,334. Such top coatings will even further reduce corrosion as well as increase the wear resistance and lower the contamination of the can contents by the oxides.

The mixed chromium oxide coating of the present invention can also be used on aluminum surfaces to form coatings that weigh from 5 to 200 milligrams per square foot. Such coatings, formed in situ as in Examples I to X inclusive, will provide greatly improved adherence for enamel, lacquer, paint or other organic layers, and will also sharply reduce the weathering of the aluminum and the resulting corrosion.

The aluminum surface that is coated according to the present invention can be either pure aluminum or so-called aluminum base alloys containing over 50% aluminum by weight. For example, the following alloys are very satisfactorily coated:

| Alloy Designations | Alloying Ingredients (in percent by weight) |
|--------------------|---------------------------------------------|
| 3S                 | 1.2 Mn.                                     |
| 52S                | 2.5 Mn, 0.25 Cr.                            |
| 61S                | 0.6 Si, 0.25 Cr, 1.0 Mg, 0.25 Cr.           |
| 24S                | 4.5 Cr, 0.6 Mn, 1.5 Mn.                     |
| 75S                |                                             |
| Alcad over 75S     | 1.0 Zn.                                     |
| 72S                |                                             |
| 62S T              |                                             |
| 17ST               | 4.0 Cr, 0.5 Mg, 0.5 Mn.                     |

The mixed chromium oxide coatings of the present invention can be applied in weights as high as 200 milligrams per square foot or higher, although little added benefit is derived from the higher weights.

The present invention is also applicable for improving the corrosion resistance and paint adhesion of aluminum-coated metals such as steel that is coated with aluminum by hot dipping, hot rolling, or electroplating. It is also very effective for aluminum foil which, when coated, makes a much better wrapping material.

The effectiveness of the coatings of the present invention appears to be greatly increased by the application of polymethylmethacrylate resin layers over the coatings. For example, a 25 to 50 milligram per square foot covering layer of polymethylmethacrylate applied from a solution of the resin in p-xylene strikingly improves the corrosion resistance of SAE 1010 steel carrying a 20 milligram per square foot coating of mixed chromium oxides in accordance with the present invention. This improvement is particularly significant where the steel is subsequently deformed, as in the making of container covers or joints. Wax type resins also show unusual cooperation with the coatings of the present invention when used in the same manner as the polymethylmethacrylate resins. Ordinary waxes and other resins are not as effective and are not even as desirable as palm oil. These resin coatings can have up to 20% plasticizer and/or pigment, and are not driven off in baking operations such as used for curing lithographic plates.

The mixed chromium oxide coating of the present invention is generally a very pale green in color with a brownish cast when the hexavalent chromium content is on the high side. However, the coating film can be colored by the addition of dyes which should be introduced into the coating film before the curing, and the dyes should be stable to the curing conditions.

Low coating weights of the mixed chromium oxide coating do not interfere with the solderability of the coating metal. For example, a 5 milligram per square foot coating on SAE 1010 steel that carries a  $\frac{1}{4}$  pound per base box tin plating, solders very readily without the use of any special flux. Heavier coatings such as 20 milligrams or more per square foot, require a special flux treatment such as that shown in application Serial No. 433,698, filed June 1, 1954. The container of Fig. 2 can be made with soldered joints, for example.

The "pound per base box" values given above are standard metal coating terms defined as the number of pounds of coating on 112 metal sheets each 14 inches by 20 inches in size.

In some cases, where metals are difficult to wet, the amount of wetting agent used may lead to foaming. This difficulty may be minimized by adding to the bath an anti-foaming agent such as water solubilized alkyl phosphate type wetting agents. For example, a 0.05% addition of monolauryl phosphate completely esterified with octaethylene glycol to a bath containing 0.3% of the wetting agent of Example I, gives very effective wetting.

The wetting problems are emphasized when the coating bath is applied by electrostatic spraying. This type of spraying is desirably carried out by whirling a film of the bath from the outer edge of a rapidly revolving cup positively charged to 90,000 volts with respect to the surface being coated.

The coating can be directed so as to produce a uniform 30 pattern by appropriately located positively charged electrodes. The bath particles are preferably whirled out at an acute angle with respect to the movement of the metal surface in the spray zone, the whirling being directed so as to follow the moving metal surface.

35 The mixed chromium oxide coatings appear to conduct electricity to some degree. When used on conductor wires they accordingly increase the current-carrying ability somewhat.

Chemical etching of aluminum for the purpose of improving the adhesion of paints or the like over the coating 40 of the present invention, is not as satisfactory if effected by etching baths such as mixtures of HF, HCl and HNO<sub>3</sub> that leave the metal surface smooth. Any alkali, even sodium carbonate, that can raise the pH of water to about 45 10, will give good etching although a pH of 11 or higher will give a much more rapid attack.

When the metal being coated in accordance with the present invention is in the form of continuous strips or the like that have to be coiled up for convenience in subsequent handling, the curing treatment is preferably followed by a rapid quench. This keeps the metal going into the coil at a sufficiently low temperature that subsequent thermal changes will not cause any trouble. Such a quench can be very simply carried out by merely passing 55 the metal, as it comes from the curing treatment, over the outer surface of a water-cooled roller. The temperature of the metal before coiling should preferably not be higher than 180° F.

The mixed chromium oxide coatings of the present invention are very good for reducing metal corrosion caused 60 by chemical influences in addition to those of ordinary weathering or handling. Chromium type stainless steels are, for example, subject to pitting and corrosion when covered with hydraulic cements or plaster of Paris, and this pitting and corrosion is practically completely prevented by the coating of the present invention. This improvement is demonstrated very forcibly with type 430 stainless steel, for instance.

The coatings of the present invention also help to reduce scaling caused by heat treatment of steel, particularly 65 when the coating of the present invention is covered by a top fused layer of inorganic protective material. Type 316 stainless steel will, by way of example, when carrying a 30 milligram per square foot coating of the present invention over which a uniform layer of borax is melted,

show no scaling whatsoever when subjected to a 2,000° F. heat treatment for one hour.

The present application is a continuation-in-part of prior applications Serial No. 278,481, filed March 25, 1952, now U.S. Patent 2,768,104, granted October 23, 1956; Serial No. 371,427, filed July 30, 1953, now U.S. Patent 2,777,785, granted January 15, 1957; and Serial No. 458,668, filed September 27, 1954, and now abandoned.

Obviously many modifications and variations of the present invention are possible in the light of the above teachings. It is, therefore, to be understood that within the scope of the appended claims the invention may be practiced otherwise than as specifically described.

What is claimed is:

1. A method for treating a non-ferrous metal surface comprising the steps of coating the surface with an aqueous solution consisting essentially of water, chromic acid and a compatible reducing agent for the chromic acid, said reducing agent being compatible with the chromic acid for at least one day at 80° F., and heating the coated surface to a temperature of from 250 to 500 degrees F. to cause the reducing agent to react with the chromic acid and leave a water-insoluble layer, the proportions of reducing agent and chromic acid being such that from about 40 to 95% of the chromium in the chromic acid is reduced to trivalent form, and the final layer weighs at least about 3 milligrams per square foot of surface.

2. The process of claim 1 in which at least about 2/3 of the chromium is reduced and the reducing agent is one that does not leave water-soluble salts in the final layer.

3. The product produced by the process of claim 2.

4. The product of claim 3 in which the metal surface is tin plated plain carbon steel in which the tin plating weighs less than 3/4 pound per base box, and the reduced chromium oxide layer weighs no more than 10 milligrams per square foot.

5. The process of claim 1 in which the metal is zinc.

6. The process of claim 1 in which the metal is aluminum.

7. The product produced by the process of claim 5.

8. The product produced by the process of claim 5 in which the metal is galvanized steel.

9. The process of claim 1 in which the metal is copper.

10. A method for treating a surface of aluminum comprising the steps of coating the surface with an aqueous solution consisting essentially of water, chromic acid and a compatible reducing agent for the chromic acid, said reducing agent being selected from the class consisting of polyalcohols and their oxidation products in which a carbon atom is linked to an alcohol group and to a hydrogen atom, and heating the coated surface to a temperature of from 250 to 500° F. to cause the reducing

agent to react with the chromic acid and leave a water-insoluble layer, the proportions of reducing agent and chromic acid being such that from about 40 to 95% of the chromium in the chromic acid is reduced to trivalent form and the final layer weighs at least about 10 milligrams per square foot of surface.

11. The product produced by the process of claim 10.

12. A method for treating a surface of galvanized steel comprising the steps of coating the galvanized surface with an aqueous solution consisting essentially of water, chromic acid and a compatible reducing agent for the chromic acid, said reducing agent being selected from the class consisting of polyalcohols and their oxidation products in which a carbon atom is linked to an alcohol group and to a hydrogen atom, and heating the coated surface to a temperature of from 250 to 500° F. to cause the reducing agent to react with the chromic acid and leave a water-insoluble layer, the proportions of reducing agent and chromic acid being such that from about 40 to 95% of the chromium in the chromic acid is reduced to trivalent form and the final layer weighs at least about 10 milligrams per square foot of surface.

13. A method for treating tin-plated steel in which the tin plating weighs less than 3/4 pound per base box, comprising the steps of coating the tin-plated surface with an aqueous solution consisting essentially of chromic acid, ammonia and a compatible reducing agent for the chromic acid, said reducing agent being compatible with the chromic acid for at least one day at 80° F., and heating the coated surface to a temperature of from 250 to 500° F. to cause the reducing agent to react with the chromic acid, and to cause the coating to be converted to a water-insoluble layer, the proportion of ammonia in the solution being such as to provide the solution with a pH between 3 and 10, and the proportions of the reducing agent and chromic acid being such that from about 40 to 95% of the chromium in the chromic acid is reduced to trivalent form, and the final layer weighs between 3 and 10 milligrams per square foot.

#### References Cited in the file of this patent

#### UNITED STATES PATENTS

|           |                 |               |
|-----------|-----------------|---------------|
| 2,315,564 | Thompson et al. | Apr. 6, 1943  |
| 2,393,640 | King            | Jan. 29, 1946 |
| 2,393,663 | Thomas et al.   | Jan. 29, 1946 |
| 2,559,812 | Watson          | July 10, 1951 |
| 2,768,104 | Schuster        | Oct. 23, 1956 |
| 2,775,535 | Poole           | Dec. 25, 1956 |
| 2,777,785 | Schuster        | June 15, 1957 |

#### FOREIGN PATENTS

|         |               |               |
|---------|---------------|---------------|
| 558,792 | Great Britain | Jan. 21, 1944 |
|---------|---------------|---------------|